

## UNITED STATES PATENT OFFICE

2,099,400

## PREPARATION OF PAPER PULP

Edwin P. Jones, Garden City, N. Y., assignor to  
 Champagne Paper Corporation, New York,  
 N. Y., a corporation of New York

No Drawing. Application October 19, 1936,  
 Serial No. 106,369

2 Claims. (Cl. 92—16)

The present invention relates to the production of a high grade bleached pulp or paper stock from flax or hemp tow.

Flax or hemp tow is now produced by a number of known chemical and/or mechanical methods or may be produced in a special decorticator. As thus produced, the tow contains approximately from 50% to 60% bast fibers, and this tow is used as the raw material from which I produce a high grade bleached pulp or paper stock by the improved method of my present invention.

As the nature of the flax or hemp straw from which the tow is produced and the chemical and/or mechanical means employed to free the same of a part of the woody matter, determines the ultimate character of the tow, the process or method employed by me in producing therefrom a high grade bleached pulp or high grade paper stock must of necessity be flexible in the method of treatment of the tow and the kind and amount of chemicals utilized in practicing the process or method. For example, if the tow contains, say, approximately 50% bast fiber, the steps of the method or process employed if the tow contains as high as, for example, 80% bast fiber, will differ specifically in minor details. Therefore while my process or method as disclosed in the present application is generic as far as the treatment of tow to produce therefrom a high grade pulp, yet the specific steps and particularly the specific quantities of chemical materials employed will of necessity vary with the character of the base material.

In carrying out my present invention the tow containing from approximately 50% to 80% bast fibers is preferably immersed in water for a sufficient time to dissolve water soluble ingredients.

The tow may be taken in the wet state and placed in a digester of conventional design, preferably a rotary digester, and cooked while being rotated under the following conditions:

(1) The amount of water used in the digester may vary between approximately 2½% to 4 times the dry weight of the fiber;

(2) The temperature during the cooking may vary from between approximately 135° and 165° centigrade, the temperature corresponding to a gauge pressure between approximately 30 and 85 pounds per square inch;

(3) The cooking time in the digester may vary between 5 to 8 hours;

(4) To the mixture of water and fiber in the digester chemicals are used constituted of a mixture of sodium hydroxide and sulphur, it being understood that the percentage of the chemicals

employed has reference to the percentage of the chemicals as based upon the dry weight of the fiber under treatment.

The chemicals employed are utilized in the following proportions based upon the dry weight of the fibers under treatment:

|                  | Percent  |
|------------------|----------|
| Sodium hydroxide | 14 to 20 |
| Sulphur          | 1 to 4   |

After the digesting operation has been completed, the digester is blown and the digested fiber is washed to remove the excess shive fiber as well as to remove the impurities in the fiber which have been rendered water soluble by the digesting process.

The washed fiber may now be suitably treated to place the pulp in a dry or semi-dry condition for storage or may be directly subjected to a bleaching process, preferably a two stage bleaching process in such a manner as to produce varying amounts of oxycellulose or related compounds, as such oxycellulose or related compounds impart special desirable properties to the paper made from the bleached pulp.

The process or method as above described produces a high grade bleached pulp from which an extremely high grade of paper may be manufactured, and in which paper there is a minimum of shives and also in which such shives as are present are invisible and which do not materially affect the grade of the paper.

The proportion of the chemicals employed are selected in accordance with the proportional content of shives in the flax tow treated.

Whereas I have described my invention by reference to specific forms thereof, it will be understood that many changes and modifications may be made without departing from the spirit of the invention.

I claim:

1. That improved method of producing bleached pulp from flax or hemp tow, which consists in subjecting the tow to a cooking operation in a digester with a solution of water of approximately 2½ to 4 times the dry weight of the fiber, and 14% to 20% sodium hydroxide and 1% to 4% sulphur, the quantities of the chemicals employed in the solution being based on the dry weight of tow; then washing the cooked fiber to remove shive fiber and water soluble impurities, and bleaching the fiber.

2. That improved method of producing bleached pulp from flax or hemp tow, which consists in dissolving water soluble materials by im-

mersing the tow in water; then subjecting the tow to a cooking operation in a digester with a solution of water of approximately 2½ to 4 times the dry weight of the fiber, and 14% to 20% sodium hydroxide and 1% to 4% sulphur, the quantities of the chemicals employed in the solu-

tion being based on the dry weight of tow; then washing the cooked fiber to remove shive fiber and water soluble impurities, and bleaching the fiber.

EDWIN P. JONES. 5